

June 16, 1931.

J. ADLER ET AL

1,810,636

TEXTILE ROLL

Filed Dec. 29, 1930



INVENTORS

Jacob Adler and  
Paul Doerseln,

BY their ATTORNEY

*John Steverns.*

## UNITED STATES PATENT OFFICE

JACOB ADLER AND PAUL DOERSELN, OF PATERSON, NEW JERSEY, ASSIGNEES TO SILK CITY METALS COATING COMPANY, INC., OF PATERSON, NEW JERSEY, A CORPORATION OF NEW JERSEY

## TEXTILE ROLL

Application filed December 29, 1930. Serial No. 505,214.

This invention has for its object to improve rolls or roll-like bodies whose peripheral surfaces are adapted to grip fibrous textile material, such as the so-called sand-roller of the 5 take-up mechanism of a loom. Such bodies are usually formed by providing a core and securing to its peripheral surface, as by glue or other cement, a covering of sand-paper. This construction is objectionable for several 10 reasons. Thus the covering itself works loose or gives way in time; its gripping action gradually becomes more and more ineffective, largely because the said particles become detached; and, which is of more serious 15 consequence, the faceted and consequently sharp angular form of the sand particles is known frequently to cut and badly damage the material gripped by the covering, particularly, as in a loom, when the weaver manipulates the fabric as an incident to the operation known as "picking back." By our invention we avoid all these objections as will appear from the following description, taken 20 with the accompanying drawings, in which 25 Fig. 1 shows a loom sand roller constructed according to the invention;

Fig. 2 is a fragmentary section thereof;

Fig. 3 shows a fragmentary section thereof on a larger scale, a certain nodular formation being magnified above the actual size usually employed; and

Fig. 4 shows a fragmentary section of a modification of the invention.

Our invention is characterized by the roll 35 or roll-like body having its periphery formed of metal and with numerous minute integral nodules which grip the fabric or other fibrous textile material placed in contact with, as extending more or less around, said periphery. These nodules are to be distinguished 40 from particles such as compose the surface of the usual sand-roller employed in loom take-up mechanisms in that, being more or less rounded protuberances and substantially wanting in sharp angles or corners such as 45 characterize the faceted particles of sand, while they are found in practice to grip the fabric or equivalent material quite as tenaciously as sand particles, they will not cut or 50 otherwise injure the material. They also

distinguish from such sand particles in that they are integral components of the surface and not secured thereto by some intermediary, as the glue or cement which binds the sand-particles of sand paper to the paper or other 55 backing or supporting sheet. When in the preferred form the roll is made up of a core and a coating of metal thereon having the nodulated gripping surface (thus permitting the core to be of a material different from 60 that of the coating) our invention is further characterized by the coating directly adhering to the core instead of being in indirect adhering relation thereto, as in the case of sand-paper secured to the core of an ordinary 65 sand-roller through the intermediary of a cementing substance.

How the roll-like body is provided with the nodulated surface is not material, but we prefer to form the body as follows:

Having a suitable core 1 (which may be wood) by a blast we discharge onto its periphery 2 a spray of fused metal particles. The particles, since they arrive at the surface in fused or molten state, adhere thereto directly, and of course as this procedure is continued to build up a metal coating 3 they become welded together to form an integral mass. When the coating has been developed to any desired thickness—which, for a body 75 to take the place of the ordinary sand-roller, need not exceed the thickness of its sand-paper coating—the application of the metal particles is stopped, and the particles of the coating which are at its exterior surface will 80 then be left set or hardened as the mentioned nodules, 4, thereon.

The durability of the surface so far as its gripping quality is concerned depends of course on the hardness of the metal of which the nodules are composed. On the other hand, we find that while certain hard metals can be fused and blasted in the form of fused particles in some cases good adhesion between 85 the coating and the core is most certainly obtained if a soft metal priming layer is first deposited on the core and then on this layer a hard metal or superficial layer having the nodules is deposited. This is shown by Fig. 100

4, where 5 indicates the priming layer and 6 the nodulated superficial layer.

Nodules as 7 in Fig. 3 are in fact formed at the inner periphery of the metal coating inset in the core where the same is of wood or other material which the molten metal particles by their heat will burn or fuse. Another feature of our invention, therefore, involves this inset condition of such nodules taken with the forming of the coating so that it surrounds and closely embraces the core, and this feature is independent of the form of the exterior or gripping surface of the coating, to wit, whether it is roughened in some way or not. A bond in such case results which insures against slippage of the coating on the core as a possible incident of expansion of the former or contraction of the latter.

Having thus fully described our invention what we claim is:

- 20 1. A roll-like body having its periphery adapted to grip textile fibrous material and formed of metal and with numerous minute integral gripping nodules.
- 25 2. A roll-like body adapted at its periphery to grip fibrous textile material and comprising a core and a coating of metal extending around and directly adhering to the core and formed at its outer periphery with numerous minute integral gripping nodules.
- 30 3. A roll-like body adapted at its periphery to grip fibrous textile material and comprising a core and a coating of metal surrounding and closely embracing the core and having its inner periphery formed with nodules inset in the core.

In testimony whereof we affix our signatures.

JACOB ADLER.  
PAUL DOERSELN.

40

45

50

55